# EUROPEAN PATENT SPECIFICATION

(11) **EP 0 695 371 B1**
(45) Date of publication and mention of the grant of the patent: **20.10.1999**
(21) Application number: 93910631.6
(22) Date of filing: 19.04.1993
(51) Int. Cl.: C22C 1/05, C25C 3/12, C25C 3/08

(54) **MICROPYRETICALLY-PRODUCED COMPONENTS OF ALUMINIUM PRODUCTION CELLS**
MIKRO-PYROTECHNISCH-ERZEUGTE BAUTEILE VON ZELLEN FUER DIE ALUMINIUMHERSTELLUNG
COMPOSANTS, PRODUITS PAR REACTION MICROPYRITIQUE, DE CELLULES DE PRODUCTION D'ALUMINIUM

(43) Date of publication of application: 07.02.1996
(73) Proprietor: MOLTECH Invent S.A., 2320 Luxembourg (LU)
(72) Inventor: SEKHAR, Jainagesh A. University of Cincinnati, Cincinnati, OH 45221-0012 (US); ZHANG, H. University of Cincinnati, Cincinnati, OH 45221-0012 (US)
(74) Representative: Cronin, Brian Harold John
(86) International application number: US9303605
(87) International publication number: WO9424321

(56) References cited:
- WO-A-92/13977
- US-A- 4 614 569
- US-A- 4 948 676

## Description

### Field of the Invention

This invention relates to components of aluminium production cells made of composite materials comprising ordered aluminide compounds of nickel, iron and/or titanium, for use in particular as anodes and cathodes and cell linings in aluminium production cells containing a fluoride-based molten electrolyte containing dissolved alumina and cerium species.

The invention is more particularly concerned with the production of components of aluminium production cells made of composite materials comprising ordered aluminide compounds of nickel, iron and/or titanium, by the micropyretic reaction of a mixture of reactive powders, which reaction mixture when ignited undergoes a micropyretic reaction to produce a net-shaped reaction product, it being understood that the reaction product may be used directly as an anode or cathode, or as substrate carrying an outer protective coating, or as a cell component.

### Background Art

US Patent N° 4,614,569 describes anodes for aluminium-production coated with a protective coating of cerium oxyfluoride, formed *in-situ* in the cell or pre-applied, this coating being maintained by the addition of cerium to the molten cryolite electrolyte. The inclusion of cerium in the substrate was proposed to promote formation of the cerium oxyfluoride coating and enhance its properties, but so far no practical way was found to effectively implement this.

US Patent N° 4,948,676 describes a ceramic/metal composite material for use as an anode for aluminium production particularly when coated with a protective cerium oxyfluoride based coating, comprising mixed oxides of cerium and one or more of aluminium, nickel, iron and copper in the form of a skeleton of interconnected ceramic oxide grains interwoven with a metallic network of an alloy or an intermetallic compound of cerium and one or more of aluminium, nickel, iron and copper. The production methods included reactive sintering, reactive hot-pressing and reactive plasma spraying of a metal powder mix optionally including some oxides. The described process conditions led to a complex porous microstructure which through dissolution and redeposition of cerium provided a self-healing effect when the anode is first used. However, difficulties were encountered in controlling the porosity of this microstructure.

US Patent N° 4,909,842 discloses the production of dense, finely grained composite materials with ceramic and metallic phases by self-propagating high temperature synthesis (SHS) with the application of mechanical pressure during or immediately after the SHS reaction. The ceramic phase may be carbides or borides of titanium, zirconium, hafnium, tantalum or niobium, silicon carbide or boron carbide. The intermetallic phase may be aluminides of nickel, titanium or copper, titanium nickelides, titanium ferrites or cobalt titanides, and the metallic phase may include aluminium, copper, nickel, iron or cobalt. The final product, which has ceramic grains in an intermetallic and/or metallic matrix, has a density of at least about 95% of the theoretical density obtained by the application of pressure. Interconnected porosity is not obtained, nor does the process control porosity. Because the pressure is applied uniaxially, it is not possible to produce a net-shaped article, i.e. whose final shape and dimensions may be largely or even completely achieved in the manufacturing process, and for which no or only minor post manufacturing processing such as grinding are required. Also, the required application of pressure prevents high production rates. Moreover, materials produced by the described method but without the application of pressure are weak and have a porosity of about 45 to 48%, which makes them unsuitable as electrodes for aluminium production.

PCT patent application WO/13977 describes the production of ceramic or ceramic-metal electrodes for electrochemical processes, in particular for aluminium production, by combustion synthesis of particulate or fibrous reactants with particulate or fibrous fillers and binders. The reactants included aluminium usually with titanium and boron; the binders included copper and aluminium; the fillers included various oxides, nitrides, borides, carbides and silicides. The described composites included copper/aluminium oxide-titanium diboride etc. This method has prospects of improved process control leading to a better microstructure, but the compositions are still in need of improvement.

PCT patent application WO/92/22682 describes an improvement of the just mentioned production method with specific fillers. The described reactants included an aluminium nickel mixture, and the binder could be a metal mixture including aluminium, nickel and up to 5 weight% copper. Among the many combinations covered is a combination of 85-90 weight% nickel-aluminium-copper with 10-15 weight% of cerium oxide. However, such combinations are very reactive and the described method does not provide details as to how to control the microstructure.

Co-pending application SN 07/861,513 discloses the production of a protective refractory coating on carbonaceous and other substrates by applying to the substrate a micropyretic reaction layer from a slurry containing particulate reactants in a colloidal carrier, and initiating a micropyretic reaction. This application is specially concerned with the production of refractory borides coatings suitable for cathodic applications.

So far, attempts to produce an electrode suitable as anode for aluminium production and based on intermetallic compounds cf aluminium with nickel, iron and/or titanium have not been successful. Additionally, no combination of such intermetallics with a ceramic has been achieved which maintains the property of a ceramic to resist oxidation at the same time achieving good conductivity at high temperatures. Moreover, attempts to incorporate cerium in an anode substrate to be coated with cerium oxyfluoride have not been successful.

### Summary of the Invention

The invention provides a method of manufacturing components of aluminium production cells made of composite materials comprising ordered aluminide compounds of nickel, iron and/or titanium, for use in particular as anodes and cathodes and cell linings in aluminium production cells containing a fluoride-based molten electrolyte containing dissolved alumina and cerium species, by micropyretic reaction of a reaction mixture comprising reactants which react to produce the aluminide-based composite material, which reaction mixture when ignited undergoes a micropyretic reaction.

According to the invention, the reaction mixture is mixed with a cerium-based colloidal carrier, dried and compacted into a reaction body bonded by the cerium-based colloid, and the colloid-bonded reaction body is ignited to initiate the micropyretic reaction. The use of a cerium-based colloidal carrier - usually colloidal ceria or cerium acetate, usually in an aqueous medium - has been found to assist bonding of the reaction mixture to form the reaction body, and contributes to moderating the micropyretic reaction as well as considerably improving the properties of the reaction product. Comparable reaction mixtures without the cerium-based colloidal carrier are difficult to bond, react poorly and do not produce a satisfactory product.

Moreover, the cerium-based colloid improves the reaction product, in particular when it is to be used as an anode for aluminium production coated with a protective cerium oxyfluoride coating. When such anode is initially immersed in a cerium-containing fluoride-based electrolyte, the colloid-originating cerium in the anode promotes initial cerium oxyfluoride formation and improves the impermeability of the cerium oxyfluoride coating by its dissolution and redeposition, which provides a self-healing effect. These effects are enhanced when the composite material of the anode also contains copper oxide. The colloid-originating cerium in the composite material also improves its performance when used as cathode or cell lining in an aluminium production cell with a cerium-containing fluoride-based electrolyte.

The cerium-based colloidal carrier may comprise colloidal ceria, colloidal cerium acetate or mixtures thereof. These cerium-based colloids may also include some colloidal silica, alumina, yttria, thoria, zirconia, magnesia, lithia or monoaluminium phosphate, and hydroxides, acetates and formates thereof as well as oxides and hydroxides of other metals, cationic species and mixtures thereof. Some particulate ceria can be included in the colloidal ceria.

The cerium-based colloid may be derived from colloid precursors and reagents which are solutions of at least one salt such as chlorides, sulfates, nitrates, chlorates, perchlorates or metal organic compounds such as alkoxides, formates, acetates The aforementioned solutions of metal organic compounds, principally metal alkoxides, may be of the general formula M(OR)_{z} where M is a metal or complex cation, R is an alkyl chain and z is a number usually from 1 to 12.

The dry colloid content of the cerium-based colloidal carrier usually corresponds to 10 - 30 weight% of the colloidal carrier, preferably 10 - 20 weight%, but may account for up to 40 weight% or even 50 weight% of the colloidal carrier, there being preferably from 10 to 20 ml of the colloidal carrier per 100 grams of the powder mixture.

The colloid-originating cerium usually amounts to 0.2 to 10% by weight of the composite material.

The reaction mixture usually comprises particulate metals from the group of aluminium, nickel, iron, titanium, copper, chromium, manganese, vanadium, molybdenum, zirconium, niobium and cerium, and/or compounds of these metals, and mixtures thereof.

A typical reaction mixture comprises 50 to 100 parts by weight of particulate nickel, iron and/or titanium and 2 to 50 parts by weight of particulate aluminium. There may also be a further 1 to 30 parts by weight of particulate additives selected from copper, chromium, manganese, vanadium, molybdenum, zirconium, niobium and cerium and compounds thereof, as well as compounds of aluminium, nickel, iron and titanium.

One preferred reaction mixture comprises 50 to 100 parts by weight of particulate nickel, 2 to 50 parts by weight of particulate aluminium and 1 to 25 parts by weight of particulate copper. Another comprises 50 to 90 parts by weight of particulate nickel, 5 to 30 parts by weight of particulate aluminium, 5 to 25 parts by weight of particulate copper and 0 to 15 parts by weight of additives selected from chromium, manganese, vanadium, molybdenum, zirconium, niobium and cerium and compounds thereof, as well as compounds of aluminium, nickel, iron, titanium and copper.

For some applications, especially for anodes, the reaction mixture includes one or more oxides of at least one metal from the group of aluminium, nickel, copper, chromium, manganese and cerium.

For cathodic applications, the reaction mixture may comprise at least one boride of at least one metal from the group titanium, chromium, vanadium, molybdenum, zirconium, niobium and cerium, or precursors that react to form said borides.

The micropyretic reaction (also called self-propagating high temperature synthesis) can be initiated by applying local heat to one or more points of the reaction body by a convenient heat source such as an electric arc, electric spark, flame, welding electrode, microwaves or laser, in which case the reaction propagates through the reaction body along a reaction front which may be self-propagating or assisted by a heat source. Reaction may also be initiated by heating the entire body to initiate reaction throughout the body in a thermal explosion mode. In either case, the reaction proceeds without supplying further heat as in a furnace. The reaction atmosphere is not critical, and reaction can take place in ambient conditions without the application of pressure.

A coating may be applied to the component produced by micropyretic reaction, the composition of this coating depending on the intended use. Such coatings may in general contain the same components as the additives listed above.

A preferred coating for aluminium-production anodes is cerium oxyfluoride according to US Patent No 4,614,569, formed *in-situ* in the cell or pre-applied. The cerium oxyfluoride may optionally contain additives such as compounds of tantalum, niobium, yttrium, tantalum, praesodymium and other rare earth elements, this coating being maintained by the addition of cerium and possibly other elements to the molten cryolite electrolyte. When a cerium oxyfluoride coating is to be applied *in-situ,* the anode substrate preferably includes cerium or cerium oxide as an additive in the composite material, in addition to the cerium from the colloidal carrier. Production of such a coating *in-situ* leads to dense and homogeneous cerium oxyfluoride. The presence of copper oxide in the anode surface is believed to enhance the cerium oxyfluoride coating.

A cathode according to the invention can also be coated with a protective refractory coating, typically containing an aluminium-wettable Refractory Hard Metal compound such as the borides and carbides of metals of Group IVB (titanium, zirconium, hafnium) and Group VB (vanadium, niobium, tantalum). Boride-containing coatings are preferred.

Such a protective coating may be formed by applying to the cathode a micropyretic reaction layer from a slurry containing particulate reactants in a colloidal carrier, and initiating a micropyretic reaction as described in co-pending application SN 07/861,513, the contents whereof are incorporated herein by way of reference. Such a micropyretic slurry comprises particulate micropyretic reactants in combination with optional particulate or fibrous non-reactant fillers or moderators in a carrier of colloidal materials or other fluids such as water or other aqueous solutions, organic carriers such as acetone, urethanes, etc., or inorganic carriers such as colloidal metal oxides.

When the cathode is coated with a refractory coating forming a cathodic surface in contact with the cathodically-produced aluminium, it can be used as a drained cathode, the refractory coating forming the cathodic surface on which the aluminium is deposited cathodically, and the component being arranged usually upright or at a slope for the aluminium to drain from the cathodic surface.

Advantageously, before use, the operative surface of the cell component is conditioned by impregnating it with colloidal ceria or cerium acetate or other colloids such as colloidal silica, alumina, yttria, thoria, zirconia, magnesia or lithia followed by drying the colloid-impregnated electrode, these impregnation/drying steps being repeated preferably until the electrode surface is saturated with the colloid. Impregnation of the component should be followed by a heat treatment and is preferably also preceded by a heat treatment. For anodes used in molten salt electrolysis, coated or not with cerium oxyfluoride, this impregnation preferably takes place with colloidal ceria or cerium acetate.

The invention also pertains to a cell component of an aluminium production cell, made of a composite material comprising at least one ordered aluminide compound of at least one of nickel, iron and titanium. The cell component is produced by micropyretic reaction of a dried reaction mixture comprising compacted particulate reactants which react to produce the composite material, bonded by a cerium-based colloidal carrier. Cerium from the colloid is dispersed in the aluminide compound forming the cell component. Usually, the colloid-originating cerium amounts to 0.2 to 10% by weight of the composite material.

A preferred composite material making up the cell component comprises nickel aluminide in solid solution with copper, and possibly also in solid solution with other metals and oxides. Another composite material comprises a major amount of Ni₃Al and minor amounts of NiAl, nickel, a ternary nickel-aluminium-copper intermetallic compound and CeO₂.

Other composite materials comprise at least one intermetallic compound from the group AlNi, AlNi₃, Al₃Fe, AlFe₃, AlTi and AlTi₃ as well as ternary intermetallic compounds derived therefrom, and solid solutions and mixtures of at least one of said intermetallic compounds with at least one of the metals aluminium, nickel, iron, titanium, copper, chromium, manganese, vanadium, molybdenum, zirconium, niobium and cerium and oxides of said metals.

Another composite material comprises an intimate mixture of at least one intermetallic compound of nickel-aluminium, at least one intermetallic compound of nickel-aluminium-copper, copper oxide, and a solid solution of at least two of the metals nickel, aluminium and copper.

The component produced by the micropyretic reaction may comprise an intimate mixture of at least one intermetallic compound of nickel-aluminium such as Ni₃Al and Al₃Ni, at least one intermetallic compound of nickel-aluminium-copper such as Al₇₃Ni₁₈Cug, copper oxide, and a solid solution of two or three metals nickel, aluminium and copper. It is believed that this material and materials like it contain non-stoichiometric conductive oxides wherein lattice vacancies are occupied by the metals or intermetallics, providing an outstanding conductivity while retaining the property of ceramic oxides to resist oxidation.

The aforementioned nickel aluminide based materials and nickel aluminide composites and solid solutions have been found to perform particularly well as dimensionally stable anodes for aluminium production.

As explained above, the cell component is advantageously impregnated with colloidal ceria, cerium acetate, silica, alumina, yttria, thoria, zirconia, magnesia or lithia.

Another aspect of the invention is a precursor of a component of an aluminium production cell which is ignitable to produce by micropyretic reaction a cell component made of a composite material comprising at least one ordered aluminide compound of at least one of nickel, iron and titanium. This precursor is a body formed of a dried reaction mixture, as explained above, comprising compacted particulate reactants which react to produce the composite material, mixed with and bonded by a cerium-based colloidal carrier. The properties of this precursor are substantially enhanced by the cerium-based colloid.

Yet another aspect of the invention is a reaction mixture for producing a component of an aluminium production cell, which component is made of a composite material comprising at least one ordered aluminide compound of at least one of nickel, iron and titanium, by micropyretic reaction of the reaction mixture after drying and compacting. The reaction mixture comprises particulate reactants, as set out above, which react to produce the composite material, mixed with a cerium-based colloidal carrier in an amount of at least 5ml of colloid per 100 grams of the reacticn mixture.

### Detailed Description

The invention will be further described in the following examples.

### Example 1

A powder mixture was prepared from nickel powder, 150 µm (-100 mesh), aluminium powder, 45 µm (-325 mesh), and copper powder, 75 µm (-200 mesh). First the nickel and aluminium powders were mixed in a ratio Ni:Al 87:13 wt%. Then this mixture was mixed with copper powder in a ratio Ni/Al:Cu 90:10 wt% in 12ml of colloidal cerium acetate per 100 grams of the powder mixture.

After 10 minutes mixing, which was sufficient to produce a good mixture, the mixture was compacted into samples by applying a pressure of about 170 MPa for 2-3 minutes, and allowed to dry in air for at least 3 hours. When the sample was almost dry, an exothermic reaction between the powders and cerium acetate occurred. To keep the samples cool and avoid cracking, cool air was blown on the samples by an air gun.

After the samples had dried completely, a small hole was drilled in the bottom of each sample to threadably receive a nickel-based superalloy rod to provide for electrical connection to the sample.

The samples were then combusted in a furnace at 900°C to initiate a micropyretic reaction which swept through the sample, and afterwards allowed to cool slowly to avoid cracking.

### Example 2

Example 1 was repeated varying the proportion of Ni:Al, in the ratios 75:25; 86.6:13.4; 90:10; 92:8; 94:6 and 96:4. The weight ratio of Ni/Al:Cu was kept constant at 90:10. Colloidal cerium acetate was added to the different series of samples in amounts of 12ml, 24ml and 36ml per 100 grams of powder mixture. Compacting was carried out at approx. 170 MPa for 4 minutes. After drying, the samples were combusted in a furnace at 950°C. All samples underwent a micropyretic reaction.

### Example 3

A sample prepared as in Example 1 was conditioned for use as an aluminium electrowinning anode by heating in air at 1000°C for 4 hours to oxidize its surface. After cooling, the sample was dipped in colloidal cerium acetate until no more is absorbed. The sample was then heated in an oven to dry it. After cooling the sample was again dipped in colloidal cerium acetate and dried. The dipping and drying steps were repeated until no more cerium acetate was absorbed.

### Example 4

A cylindrical piece of 25 mm diameter and 40 mm height was prepared using the micropyretic technique of Example 2, with the composition Ni:Al 86.6:13.4, mixed with colloidal cerium acetate in an amount of 24ml/100 grams of the powder mixture. The material was then submitted to a heat treatment in air at 1000°C for 10 hours. The weight uptake due to oxidation was about 6%. The oxidized material was impregnated by dipping into a colloidal solution of cerium acetate for 10 minutes and drying at 250°C. This operation was repeated twice. The sample was then tested as an anode in a small electrolytic cell containing molten cryolite at 1000°C with 5% alumina and 1.5% cerium fluoride, at a current density of 0.3 A/cm² for 4 hours. The cell voltage remained stable at 4V during the test. The test anode was then cross-sectioned and no significant corrosion was observed.

### Example 5

The same pretreatment and test procedures were applied to a second sample with the composition Ni:Al 90:10 mixed with colloidal cerium acetate in an amount of 24ml per 100 grams of the powder mixture. The test results were similar to the previous material.

### Example 6

The same pretreatment and test procedures were applied to a third sample with the composition Ni:Al 90:10 but mixed with colloidal cerium acetate in an amount of 36ml per 100 grams of the powder mixture. The weight uptake after the heat treatment was more important (about 20% greater) but the material did not show any crack or fissure. The electrolytic test gave results similar to the previous examples with a somewhat higher cell voltage of 5 Volts.

### Example 7

The previous examples were repeated varying the size of the particulate nickel (1 to 10 micrometer diameter), copper (1 to 100 micrometer diameter) and aluminium (1 to 100 micrometer diameter). Best results in terms of lowest porosity and electrochemical performance were obtained with nickel 3 micrometer diameter, copper 10 micrometer diameter and aluminium 44 micrometer diameter (-325 mesh).

### Example 8

The previous examples were repeated replacing the colloidal cerium acetate with colloidal ceria optionally containing some ceria powder. Excellent results were obtained.

## Claims

1. A method of manufacturing components of aluminium production cells made of composite materials comprising ordered aluminide compounds of at least one of nickel, iron and titanium, by micropyretic reaction of a reaction mixture comprising compacted particulate reactants which react to produce the composite material, wherein the reaction mixture is mixed with a cerium-based colloidal carrier, dried and compacted into a reaction body bonded by the cerium-based colloidal carrier, and the colloid-bonded reaction body is ignited to initiate the micropyretic reaction.

2. The method of claim 1, wherein the cerium-based colloidal carrier comprises at least one of colloidal ceria and colloidal cerium acetate.

3. The method of claim 2, wherein the cerium-based colloidal carrier further comprises at least one of colloidal alumina, yttria, silica, thoria, zirconia, magnesia, lithia or monoaluminium phosphate.

4. The method of claim 2, wherein the cerium-based colloidal carrier is derived from colloid precursors and reagents which are solutions of at least one salt such as chlorides, sulfates, nitrates, chlorates, perchlorates or metal organic compounds such as alkoxides, formates, acetates and mixtures thereof.

5. The method of claim 4, wherein the solutions of metal organic compounds, principally metal alkoxides, are of the general formula M(OR)_{z} where M is a metal or complex cation, R is an alkyl chain and z is a number usually from 1 to 12.

6. The method of claim 2, wherein the cerium-based colloidal carrier has a dry colloid content corresponding to up to 50 weight% of the colloidal carrier, preferably from 10 to 20 weight%, there being from 10 to 20 ml of the colloidal carrier per 100 grams of the reaction mixture.

7. The method of claim 1, wherein the reaction mixture comprises particulate metals or compounds of metals selected from the group consisting of aluminium, nickel, iron, titanium, copper, chromium, manganese, vanadium, molybdenum, zirconium, niobium and cerium, and mixtures thereof.

8. The method of claim 7, wherein the reaction mixture comprises 50 to 100 parts by weight of at least one of particulate nickel, iron and titanium and 2 to 50 parts by weight of particulate aluminium.

9. The method of claim 8, wherein the reaction mixture further comprises 1 to 30 parts by weight of particulate additives selected from copper, chromium, manganese, vanadium, molybdenum, zirconium, niobium and cerium and compounds thereof as well as compounds of aluminium, nickel, iron and titanium.

10. The method of claim 9, wherein the reaction mixture comprises 50 to 100 parts by weight of particulate nickel, 2 to 50 parts by weight of particulate aluminium and 1 to 25 parts by weight of particulate copper.

11. The method of claim 10, wherein the reaction mixture comprises 50 to 90 parts by weight of particulate nickel, 5 to 30 parts by weight of particulate aluminium, 5 to 25 parts by weight of particulate copper and 0 to 15 parts by weight of additives selected from chromium, manganese, vanadium, molybdenum, zirconium, niobium and cerium and compounds thereof as well as compounds of aluminium, nickel, iron, titanium and copper.

12. The method of claim 9, wherein the reaction mixture comprises at least one oxide of at least one metal from the group of aluminium, nickel, copper, chromium, manganese and cerium.

13. The method of claim 9, wherein the reaction mixture comprises at least one boride of at least one metal from the group titanium, chromium, vanadium, zirconium, niobium and cerium, or precursors that react to form said borides.

14. The method of claim 1, wherein the composite material comprises at least one intermetallic compound from the group AlNi, AlNi₃, Al₃Fe, AlFe₃, AlTi and AlTi₃ as well as ternary intermetallic compounds derived therefrom, and solid solutions and mixtures of at least one of said intermetallic compounds with at least one of the metals aluminium, nickel, iron, titanium, copper, chromium, manganese, vanadium, molybdenum, zirconium, niobium and cerium and oxides of said metals.

15. The method of claim 1, wherein the colloid-originating cerium amounts to 0.2 to 10% by weight of the composite material.

16. The method of claim 1, comprising applying a coating onto a surface of the composite material formed by said micropyretic reaction.

17. The method of claim 16, wherein the component is a cathode and the surface coating comprises a Refractory Hard Metal boride.

18. The method of claim 16, wherein the component is an anode and the surface coating comprises at least one rare earth oxycompound including cerium oxyfluoride.

19. The method of claim 1, further comprising impregnating the operative surface of the component with colloidal ceria, cerium acetate, silica, alumina, yttria, thoria, zirconia, magnesia or lithia and drying the colloid-impregnated electrode.

20. The method of claim 19, wherein impregnation of the component is followed by a heat treatment and is preferably also preceded by a heat treatment.

21. The method of claim 19 or 20, wherein the impregnation and the drying steps are repeated until the electrode surface is saturated with the colloid.

22. A cell component of an aluminium production cell which component is made of a composite material comprising at least one ordered aluminide compound of at least one of nickel, iron and titanium produced by micropyretic reaction of a dried reaction mixture comprising compacted particulate reactants which react to produce the composite material, bonded by a cerium-based colloidal carrier, the cell component comprising cerium from the colloid dispersed in the aluminide compound.

23. The cell component of claim 22, wherein the composite material comprises nickel aluminide in solid solution with copper.

24. The cell component of claim 22, wherein the composite material comprises a major amount of Ni₃Al and minor amounts of NiAl, nickel, a ternary nickel-aluminium-copper intermetallic compound and CeO₂.

25. The cell component of claim 22, wherein the composite material comprises at least one intermetallic compound from the group AlNi, AlNi₃, Al₃Fe, AlFe₃, AlTi and AlTi₃ as well as ternary intermetallic compounds derived therefrom, and solid solutions and mixtures of at least one of said intermetallic compounds with at least one of the metals aluminium, nickel, iron, titanium, copper, chromium, manganese, vanadium, molybdenum, zirconium, niobium and cerium and oxides of said metals.

26. The cell component of claim 22, wherein the composite material comprises an intimate mixture of at least one intermetallic compound of nickel-aluminium, at least one intermetallic compound of nickel-aluminium-copper, copper oxide, and a solid solution of at least two of the metals nickel, aluminium and copper.

27. The cell component of claim 22, which is an anode coated with cerium oxyfluoride.

28. The cell component of claim 22, which is a cathode coated with or containing at least one Refractory Hard Metal Boride.

29. The cell component of claim 22, which is impregnated with colloidal ceria, cerium acetate, silica, alumina, yttria, thoria, zirconia, magnesia or lithia.

30. The cell component of claim 22, wherein the colloid-originating cerium amounts to 0.2 to 10% by weight of the composite material.

31. A precursor of a component of an aluminium production cell which is ignitable to produce by micropyretic reaction a cell component made of a composite material comprising at least one ordered aluminide compound of at least one of nickel, iron and titanium, wherein the precursor is formed of a dried reaction mixture comprising compacted particulate reactants which react to produce the composite material, the compacted particulate reactants being mixed with and bonded by a cerium-based colloidal carrier.

32. The precursor of claim 31, wherein the cerium-based colloidal carrier comprises at least one of colloidal ceria and colloidal cerium acetate.

33. The precursor of claim 32, wherein the cerium-based colloidal carrier further comprises at least one of colloidal alumina, yttria, silica, thoria, zirconia, magnesia, lithia or monoaluminium phosphate.

34. The precursor of claim 31, obtained by drying a cerium-based colloidal carrier having a dry colloid content corresponding to up to 50 weight% of the colloidal carrier, preferably from 10 to 20 weight%, there being from 10 to 20 ml of the colloidal carrier per 100 grams of the reaction mixture.

35. The precursor of claim 31, wherein the reaction mixture comprises particulate metals or compounds of metals selected from the group consisting of aluminium, nickel, iron, titanium, copper, chromium, manganese, vanadium, molybdenum, zirconium, niobium and cerium, and mixtures thereof.

36. The precursor of claim 32, wherein the reaction mixture comprises 50 to 100 parts by weight of at least one of particulate nickel, iron and titanium and 2 to 50 parts by weight of particulate aluminium.

37. The precursor of claim 36, wherein the reaction mixture further comprises 1 to 30 parts by weight of particulate additives selected from copper, chromium, manganese, vanadium, molybdenum, zirconium, niobium and cerium and compounds thereof as well as compounds of aluminium, nickel, iron and titanium.

38. The precursor of claim 37, wherein the reaction mixture comprises 50 to 100 parts by weight of particulate nickel, 2 to 50 parts by weight of particulate aluminium and 1 to 25 parts by weight of particulate copper.

39. The precursor of claim 38, wherein the reaction mixture comprises 50 to 90 parts by weight of particulate nickel, 5 to 30 parts by weight of particulate aluminium, 5 to 25 parts by weight of particulate copper and 0 to 15 parts by weight of additives selected from chromium, manganese, vanadium, molybdenum, zirconium, niobium and cerium and compounds thereof as well as compounds of aluminium, nickel, iron, titanium and copper.

40. The precursor of claim 37, wherein the reaction mixture comprises at least one oxide of at least one metal from the group of aluminium, nickel, copper, chromium, manganese and cerium.

41. The precursor of claim 37, wherein the reaction mixture comprises at least one boride of at least one metal from the group titanium, chromium, vanadium, zirconium, niobium and cerium, or precursors that react to form said borides.

42. The precursor of claim 31, wherein the composite material comprises at least one intermetallic compound from the group AlNi, AlNi₃, Al₃Fe, AlFe₃, AlTi and AlTi₃ as well as ternary intermetallic compounds derived therefrom, and solid solutions and mixtures of at least one of said intermetallic compounds with at least one of the metals aluminium, nickel, iron, titanium, copper, chromium, manganese, vanadium, molybdenum, zirconium, niobium and cerium and oxides of said metals.

43. The precursor of claim 31, wherein the colloid-originating cerium amounts to 0.2 to 10% by weight of the composite material.

44. A reaction mixture for producing a component of an aluminium production cell, which component is made of a composite material comprising at least one ordered aluminide compound of at least one of nickel, iron and titanium, by micropyretic reaction of the reaction mixture after drying and compacting, the reaction mixture comprising particulate reactants which react to produce the composite material mixed with a cerium-based colloidal carrier in an amount of at least 5ml of colloid per 100 grams of the reaction mixture.

## Patentansprüche

1. Verfahren zur Herstellung von Komponenten von Aluminiumproduktionszellen, die aus Kompositmaterialien hergestellt sind, die geordnete Aluminidverbindungen von zumindest einem von Nickel, Eisen und Titan enthalten, durch mikro-pyrotechnische Reaktion von einem Reaktionsgemisch, das kompakte partikuläre Reaktanten enthält, die reagieren, um das Kompositmaterial zu produzieren, wobei das Reaktionsgemisch mit einem auf Cer basierenden, kolloidalen Trägerstoff gemischt, getrocknet und zu einem Reaktionskörper komprimiert wird, der durch den auf Cer basierenden, kolloidalen Trägerstoff gebunden ist, und der kolloidal gebundene Reaktionskörper entzündet wird, um die mikro-pyrotechnische Reaktion einzuleiten.

2. Verfahren nach Anspruch 1, bei dem der auf Cer basierende, kolloidale Trägerstoff zumindest eines von kolloidalem Ceroxid und kolloidalem Ceracetat enthält.

3. Verfahren nach Anspruch 2, bei dem der auf Cer basierende, kolloidale Trägerstoff außerdem zumindest eines von kolloidalem Aluminiumoxid, Yttriumoxid, Siliciumdioxid, Thoriumdioxid, Zirkoniumdioxid, Magnesiumoxid, Lithiumoxid oder Monoaluminiumphosphat enthält.

4. Verfahren nach Anspruch 2, bei dem der auf Cer basierende, kolloidale Trägerstoff von kolloidalen Vorläufern und Reagenzien abstammt, die Lösungen zumindest eines Salzes, wie Chloride, Sulfate, Nitrate, Chlorate, Perchlorate, oder metallorganische Verbindungen sind, wie Alkoxide, Formate, Acetate und Mischungen davon.

5. Verfahren nach Anspruch 4, bei dem die Lösungen der metallorganischen Verbindungen, im wesentlichen Metallalkoxide, mittels der allgemeinen Formel M(OR)_{z} darstellbar sind, bei der M ein Metall- oder Komplex-Kation, R eine Alkylkette und z eine Zahl normalerweise von 1 bis 12 ist.

6. Verfahren nach Anspruch 2, bei dem der auf Cer basierende, kolloidale Trägerstoff einen trockenen kolloidalen Anteil hat, der bis zu 50 Gew.-% des kolloidalen Trägerstoffs entspricht, vorzugsweise von 10 bis 20 Gew.-%, wobei 10 bis 20 ml des kolloidalen Trägerstoffes pro 100 g des Reaktionsgemisches vorliegen.

7. Verfahren nach Anspruch 1, bei dem das Reaktionsgemisch partikuläre Metalle oder Verbindungen von Metallen enthält, die aus der Gruppe ausgewählt sind, die Aluminium, Nickel, Eisen, Titan, Kupfer, Chrom, Mangan, Vanadium, Molybdän, Zirkonium, Niob und Cer sowie Mischungen davon umfaßt.

8. Verfahren nach Anspruch 7, bei dem das Reaktionsgemisch 50 bis 100 Gewichtsanteile von zumindest einem von partikulärem Nickel, Eisen oder Titan sowie 2 bis 50 Gewichtsanteile von partikulärem Aluminium enthält.

9. Verfahren nach Anspruch 8, bei dem das Reaktionsgemisch außerdem 1 bis 30 Gewichtsanteile von partikulären Zusatzstoffen, die aus Kupfer, Chrom, Mangan, Vanadium, Molybdän, Zirkonium, Niob und Cer sowie Verbindungen davon ausgewählt sind, und auch Verbindungen von Aluminium, Nickel, Eisen und Titan enthält.

10. Verfahren nach Anspruch 9, bei dem das Reaktionsgemisch 50 bis 100 Gewichtsanteile von partikulärem Nickel, 2 bis 50 Gewichtsanteile von partikulärem Aluminium und 1 bis 25 Gewichtsanteile von partikulärem Kupfer enthält.

11. Verfahren nach Anspruch 10, bei dem das Reaktionsgemisch 50 bis 90 Gewichtsanteile von partikulärem Nickel, 5 bis 30 Gewichtsanteile von partikulärem Aluminium, 5 bis 25 Gewichtsanteile von partikulärem Kupfer und 0 bis 15 Gewichtsanteile von Zusatzstoffen, die aus Chrom, Mangan, Vanadium, Molybdän, Zirkonium, Niob und Cer sowie Verbindungen davon ausgewählt sind, und auch Verbindungen von Aluminium, Nickel, Eisen, Titan und Kupfer enthält.

12. Verfahren nach Anspruch 9, bei dem das Reaktionsgemisch zumindest ein Oxid von zumindest einem Metall aus der Gruppe von Aluminium, Nickel, Kupfer, Chrom, Mangan und Cer enthält.

13. Verfahren nach Anspruch 9, bei dem das Reaktionsgemisch zumindest ein Borid von zumindest einem Metall aus der Gruppe von Titan, Chrom, Vanadium, Zirkonium, Niob und Cer, oder Vorläufer enthält, die reagieren, um diese Boride zu bilden.

14. Verfahren nach Anspruch 1, bei dem das Kompositmaterial zumindest eine intermetallische Verbindung aus der Gruppe von AlNi, AlNi₃, Al₃Fe, AlFe₃, AlTi und AlTi₃ sowie auch ternäre intermetallische Verbindungen, die davon abstammen, und feste Lösungen und Mischungen aus zumindest einem der intermetallischen Bestandteile mit zumindest einem der Metalle Aluminium, Nickel, Eisen, Titan, Kupfer, Chrom, Mangan, Vanadium, Molybdän, Zirkonium, Niob und Cer sowie Oxiden dieser Metalle enthält.

15. Verfahren nach Anspruch 1, bei dem sich das aus Kolloid stammende Cer auf 0,2 bis 10 Gew.-% des Kompositmaterials beläuft.

16. Verfahren nach Anspruch 1, bei dem eine Beschichtung auf eine Oberfläche des Kompositmaterials aufgebracht wird, das durch die mikro-pyrotechnische Reaktion gebildet wurde.

17. Verfahren nach Anspruch 16, bei dem die Komponente eine Kathode ist und die Oberflächenbeschichtung ein feuerfestes Hartmetallborid enthält.

18. Verfahren nach Anspruch 16, bei dem die Komponente eine Anode ist und die Oberflächenbeschichtung zumindest einen Seltenerdmetalloxybestandteil enthält, einschließlich Ceroxyfluorid.

19. Verfahren nach Anspruch 1, außerdem mit dem Imprägnieren der operativen Oberfläche der Komponente mit kolloidalem Cer, Ceracetat, Siliciumdioxid, Aluminiumoxid, Yttriumoxid, Thoriumdioxid, Zirkoniumdioxid, Magnesiumoxid oder Lithiumoxid sowie dem Trocknen der kolloid-imprägnierten Elektrode.

20. Verfahren nach Anspruch 19, bei dem auf das Imprägnieren der Komponente eine Hitzebehandlung folgt und ersterem vorzugsweise ebenfalls eine Hitzebehandlung vorausgeht.

21. Verfahren nach Anspruch 19 oder 20, bei dem die Schritte des Imprägnierens und Trocknens wiederholt werden, bis die Elektrodenoberfläche mit dem Kolloid gesättigt ist.

22. Zellenkomponente einer Aluminiumproduktionszelle, bei der die Komponente aus einem Kompositmaterial hergestellt ist, das zumindest eine geordnete Aluminidverbindung von zumindest einem von Nickel, Eisen und Titan enthält, die durch mikro-pyrotechnische Reaktion von einem getrockneten Reaktionsgemisch produziert ist, das kompakte partikuläre Reaktanten enthält, die reagieren, um das Kompositmaterial zu produzieren, gebunden durch einen auf Cer basierenden, kolloidalen Trägerstoff, wobei die Zellenkomponente Cer aus dem in der Aluminidverbindung dispergierten Kolloid enthält.

23. Zellenkomponente nach Anspruch 22, bei der das Kompositmaterial Nickelaluminid in fester Lösung mit Kupfer enthält.

24. Zellenkomponente nach Anspruch 22, bei der das Kompositmaterial eine größere Menge an Ni₃Al und geringere Mengen an NiAl, Nickel, einer ternären intermetallischen Nickel/ Aluminium/Kupfer-Verbindung und CeO₂ enthält.

25. Zellenkomponente nach Anspruch 22, bei der das Kompositmaterial zumindest eine intermetallische Verbindung aus der Gruppe von AlNi, AlNi₃, Al₃Fe, AlFe₃, AlTi und AlTi₃ und auch davon abstammende, ternäre intermetallische Verbindungen sowie feste Lösungen und Mischungen von zumindest einer der intermetallischen Verbindungen mit zumindest einem der Metalle Aluminium, Nickel, Eisen, Titan, Kupfer, Chrom, Mangan, Vanadium, Molybdän, Zirkonium, Niob und Cer sowie Oxiden dieser Metalle enthält.

26. Zellenkomponente nach Anspruch 22, bei der das Kompositmaterial eine innige Mischung aus zumindest einer intermetallischen Verbindung von Nickel/Aluminium, zumindest einer intermetallischen Verbindung von Nickel/Aluminium/Kupfer, Kupferoxid und einer festen Lösung von zumindest zwei der Metalle Nickel, Aluminium und Kupfer enthält.

27. Zellenkomponente nach Anspruch 22, die eine mit Ceroxyfluorid beschichtete Anode ist.

28. Zellenkomponente nach Anspruch 22, die eine Kathode ist, die mindestens mit einem feuerfesten Hartmetallborid beschichtet ist oder zumindest ein solches enthält.

29. Zellenkomponente nach Anspruch 22, die mit kolloidalem Cer, Ceracetat, Siliciumdioxid, Aluminiumoxid, Yttriumoxid, Thoriumdioxid, Zirkoniumdioxid, Magnesiumoxid oder Lithiumoxid imprägniert ist.

30. Zellenkomponente nach Anspruch 22, bei der sich das aus Kolloid stammende Cer auf 0,2 bis 10 Gew.-% des Kompositmaterials beläuft.

31. Vorläufer einer Komponente einer Aluminiumproduktionszelle, der entzündlich ist, um durch eine mikro-pyrotechnische Reaktion eine Zellenkomponente herzustellen, die aus einem Kompositmaterial hergestellt ist, das zumindest eine geordnete Aluminidverbindung von zumindest einem von Nickel, Eisen und Titan enthält, wobei der Vorläufer aus einem trockenen Reaktionsgemisch hergestellt ist, das kompakte partikuläre Reaktanten enthält, die reagieren, um das Kompositmaterial zu produzieren, wobei die kompakten partikulären Reaktanten mit einem auf Cer basierenden, kolloidalen Trägerstoff gemischt und an diesen gebunden sind.

32. Vorläufer nach Anspruch 31, bei dem der auf Cer basierende, kolloidale Trägerstoff zumindest eines von kolloidalem Ceroxid und kolloidalem Ceracetat enthält.

33. Vorläufer nach Anspruch 32, bei dem der auf Cer basierende, kolloidale Trägerstoff außerdem zumindest eines von kolloidalem Aluminiumoxid, Yttriumoxid, Siliciumdioxid, Thoriumdioxid, Zirkoniumdioxid, Magnesiumoxid, Lithiumoxid oder Monoaluminiumphosphat enthält.

34. Vorläufer nach Anspruch 31, der durch Trocknen eines auf Cer basierenden, kolloidalen Trägerstoffes erhalten wird, der einen trockenen kolloidalen Anteil hat, der bis zu 50 Gew.-% des kolloidalen Trägerstoffes entspricht, vorzugsweise von 10 bis 20 Gew.-%, wobei 10 bis 20 ml des kolloidalen Trägerstoffes pro 100 g des Reaktionsgemisches vorliegen.

35. Vorläufer nach Anspruch 31, bei dem das Reaktionsgemisch partikuläre Metalle oder Metallverbindungen enthält, die aus der Gruppe ausgewählt sind, die Aluminium, Nickel, Eisen, Titan, Kupfer, Chrom, Mangan, Vanadium, Molybdän, Zirkonium, Niob und Cer sowie Mischungen davon enthält.

36. Vorläufer nach Anspruch 32, bei dem das Reaktionsgemisch 50 bis 100 Gewichtsanteile von zumindest einem aus partikulärem Nickel, Eisen und Titan sowie 2 bis 50 Gewichtsanteile von partikulärem Aluminium enthält.

37. Vorläufer nach Anspruch 36, bei dem das Reaktionsgemisch außerdem 1 bis 30 Gew.-% von partikulären Zusatzstoffen, die aus Kupfer, Chrom, Mangan, Vanadium, Molybdän, Zirkonium, Niob und Cer sowie Verbindungen davon ausgewählt sind, und auch Verbindungen von Aluminium, Nickel, Eisen und Titan enthält.

38. Vorläufer nach Anspruch 37, bei dem das Reaktionsgemisch 50 bis 100 Gewichtsanteile von partikulärem Nickel, 2 bis 50 Gewichtsanteile von partikulärem Aluminium und 1 bis 25 Gewichtsanteile von partikulärem Kupfer enthält.

39. Vorläufer nach Anspruch 38, bei dem das Reaktionsgemisch 50 bis 90 Gewichtsanteile von partikulärem Nickel, 5 bis 30 Gewichtsanteile von partikulärem Aluminium, 5 bis 25 Gewichtsanteile von partikulärem Kupfer und 0 bis 15 Gewichtsanteile von Zusatzstoffen, die aus Chrom, Mangan, Vanadium, Molybdän, Zirkonium, Niob und Cer und Verbindungen davon ausgewählt sind, und auch Verbindungen von Aluminium, Nickel, Eisen, Titan und Kupfer enthält.

40. Vorläufer nach Anspruch 37, bei dem das Reaktionsgemisch zumindest ein Oxid von zumindest einem Metall aus der Gruppe Aluminium, Nickel, Kupfer, Chrom, Mangan und Cer enthält.

41. Vorläufer nach Anspruch 37, bei dem das Reaktionsgemisch zumindest ein Borid von zumindest einem Metall aus der Gruppe Titan, Chrom, Vanadium, Zirkonium, Niob und Cer, oder Vorläufer enthält, die reagieren, um die Boride zu bilden.

42. Vorläufer nach Anspruch 31, bei dem das Kompositmaterial zumindest eine intermetallische Verbindung aus der Gruppe AlNi, AlNi₃, Al₃fe, Alfe₃, AlTi und AlTi₃ sowie davon abstammende ternäre intermetallische Verbindungen, sowie auch feste Lösungen und Mischungen von zumindest einer intermetallischen Verbindung mit zumindest einem der Metalle Aluminium, Nickel, Eisen, Titan, Kupfer, Chrom, Mangan, Vanadium, Molybdän, Zirkonium, Niob und Cer sowie Oxide dieser Metalle enthält.

43. Vorläufer nach Anspruch 31, bei dem sich das aus Kolloid stammende Cer auf 0,2 bis 10 Gew.-% des Kompositmaterials beläuft.

44. Reaktionsgemisch zur Produktion einer Komponente einer Aluminiumproduktionszelle, wobei die Komponente aus einem Kompositmaterial hergestellt ist, das zumindest eine geordnete Aluminidverbindung von zumindest einem von Nickel, Eisen oder Titan enthält, durch mikro-pyrotechnische Reaktion des Reaktionsgemisches nach Trocknen und Komprimieren, wobei das Reaktionsgemisch partikuläre Reaktanten enthält, die reagieren, um das Kompositmaterial zu produzieren, das mit einem auf Cer basierenden, kolloidalen Trägerstoff in einer Menge von zumindest 5 ml des Kolloids pro 100 g des Reaktionsgemisches gemischt ist.

## Revendications

1. Méthode de fabrication de composants de cellules de production d'aluminium faites en matériaux composites comprenant des composés d'aluminure ordonnés d'au moins un parmi le nickel, le fer, et le titane, par réaction micropyrétique d'un mélange de réaction comprenant des réactifs particulaires compactés qui réagissent pour produire le matériau composite, dans lequel le mélange de réaction est mélangé avec un porteur colloïdal à base de cérium, séché et compacté dans un corps de réaction lié par le porteur colloïdal à base de cérium, et le corps de réaction lié par le colloïde est allumé pour initier le réaction micropyrétique.

2. La méthode de la revendication 1, dans laquelle le porteur colloïdal à base de cérium comprend au moins un parmi l'oxyde de cérium colloïdal et l'acétate de cérium colloïdal.

3. La méthode de la revendication 2, dans laquelle le porteur colloïdal à base de cérium comprend au moins un parmi l'alumine, l'oxyde d'yttrium, la silice, l'oxyde de thorium, l'oxyde de zirconium, l'oxyde de magnésium, l'oxyde de lithium ou le monoaluminium phosphate colloïdaux.

4. La méthode de la revendication 2, dans laquelle le porteur colloïdal à base de cérium est dérivé de précurseurs colloïdaux et les réactifs qui sont des solutions d'au moins un sel comme les chlorure, sulfates, nitrates, chlorates, ou les composés métal-organiques comme les alkoxydes, les formates, les acétates et leurs mélanges.

5. La méthode de la revendication 4, dans laquelle les solutions de composés métal-organique, principalement les alkoxydes de métaux, sont de formule générale M(OR)_{z} où M est un métal ou un cation complexe, R est une chaîne alkyle et z est un nombre habituellement de 1 à 12.

6. La méthode de la revendication 2, dans laquelle le porteur colloïdal à base de cérium a un contenu colloïde sec correspondant à jusqu'à 50 % en poids de porteur colloïdal, préférablement de 10 à 20 % en poids, ayant ainsi de 10 à 20 ml de porteur colloïdal par 100 grammes de mélange de réaction.

7. La méthode de la revendication 1, dans laquelle le mélange de réaction comprend des métaux particulaires ou des composés de métaux sélectionnés du groupe consistant de l'aluminium, du nickel, du fer, du titane, du cuivre, du chrome, du manganèse, du vanadium, du molybdène, du zirconium, du niobium et du cérium, et leurs mélanges.

8. La méthode de la revendication 7, dans laquelle le mélange de réaction comprend de 50 à 100 parts en poids d'au moins un parmi le nickel, le fer, et le titane particulaires, et de 2 à 50 parts en poids d'aluminium particulaire.

9. La méthode de la revendication 8, dans laquelle le mélange de réaction comprend de 1 à 30 parts en poids d'additifs particulaires sélectionnés parmi le cuivre, le chrome, le manganèse, le vanadium, le molybdène, le zirconium, le niobium et le cérium et leurs composés ainsi que des composés d'aluminium, de nickel, de fer et de titane.

10. La méthode de la revendication 9, dans laquelle le mélange de réaction comprend de 50 à 100 parts en poids de nickel particulaire, de 2 à 50 parts en poids d'aluminium particulaire et de 1 à 25 parts en poids de cuivre particulaire.

11. La méthode de la revendication 10, dans laquelle le mélange de réaction comprend de 50 à 90 parts en poids de nickel particulaire, de 5 à 30 parts en poids d'aluminium particulaire, de 5 à 25 parts en poids de cuivre particulaire et de 0 à 15 parts en poids d'additifs sélectionnés parmi le chrome, le manganèse, le vanadium, le molybdène, le zirconium, le niobium et le cérium et leurs composés ainsi que les composés d'aluminium de nickel, de fer, de titane et de cuivre.

12. La méthode de la revendication 9, dans laquelle le mélange de réaction comprend au moins un oxyde d'au moins un métal du groupe de l'aluminium, du nickel, du cuivre, du chrome, du manganèse et du cérium.

13. La méthode de la revendication 9, dans laquelle le mélange de réaction comprend au moins un métal du groupe du titane, du chrome, du vanadium, du zirconium, du niobium et du cérium, ou des précurseurs qui réagissent pour former lesdits borures.

14. La méthode de la revendication 1, dans laquelle le matériau composite comprend au moins un composé intermétallique du groupe du AlNi, AlNi₃, Al₃Fe, AlFe₃, AlTi et AlTi₃ ainsi que leurs composés intermétalliques ternaires dérivés, et les solutions et mélanges solides d'au moins un desdits composés intermétalliques avec au moins un des métaux parmi l'aluminium, le nickel, le fer, le titane, le cuivre, le chrome, le manganèse, le vanadium, le molybdène, le zirconium, le niobium et le cérium et les oxydes desdits métaux.

15. La méthode de la revendication 1, dans laquelle le cérium provenant du colloïde représente de 0,2 à 10 % en poids du matériau composite.

16. La méthode de la revendication 1, comprenant l'application d'un revêtement sur une surface du matériau composite formé par ladite réaction micropyrétique.

17. La méthode de la revendication 16, dans laquelle le composant est une cathode et le revêtement de surface comprend un borure de Métal réfractaire dur.

18. La méthode de la revendication 16, dans laquelle le composant est une anode et la surface du revêtement comprend au moins un oxycomposé de terre rare y compris l'oxyfluorure de cérium.

19. La méthode de la revendication 1, comprenant en plus l'imprégnation de la surface opérative du composant avec de l'oxyde de cérium, de l'acétate de cérium, de la silice, de l'alumine, de l'oxyde d'yttrium, de l'oxyde de thorium, de l'oxyde de zirconium, de l'oxyde de magnésium, ou de l'oxyde de lithium colloïdaux et le séchage de l'électrode imprégnée de colloïde.

20. La méthode de la revendication 19, dans laquelle l'imprégnation du composant est suivie par un traitement à la chaleur et est aussi précédée préférablement par un traitement à la chaleur.

21. La méthode de la revendication 19 ou 20, dans laquelle les étapes d'imprégnation et de séchage sont répétées jusqu'à ce que la surface de l'électrode soit saturée de colloïde.

22. Composant de cellule d'une cellule de production d'aluminium dont le composant est réalisé avec un matériau composite comprenant au moins un composé d'aluminure ordonné d'au moins un parmi le nickel, le fer et le titane produit par réaction micropyrétique d'un mélange de réaction séché comprenant des réactifs particulaires compactés qui réagissent pour produire le matériau composite, lié par un porteur colloïdal à base de cérium, le composant de cellule comprenant du cérium à partir du colloïde dispersé dans le composé d'aluminure.

23. Le composant de cellule de la revendication 22, dans lequel le matériau composite comprend de l'aluminure de nickel en solution solide avec du cuivre.

24. Le composant de cellule de la revendication 22, dans lequel le matériau composite comprend une quantité majeure de Ni₃Al et des quantités mineures de NiAl, de nickel, d'un composé intermétallique ternaire nickel-aluminium-cuivre et de CeO₂.

25. Le composant de cellule de la revendication 22, dans lequel le matériau composite comprend au moins un composé intermétallique du groupe du AlNi, AlNi₃, AL₃Fe, AlFe₃, AlTi et AlTi₃ ainsi que des composés intermétalliques ternaires dérivés de ceux-ci, et des solutions solides et des mélanges d'au moins un desdits composés intermétalliques avec au moins un des métaux parmi l'aluminium, le nickel, le fer, le titane, le cuivre, le chrome, le manganèse, le vanadium, le molybdène, le zirconium, le niobium et le cérium et leurs oxydes.

26. Le composant de cellule de la revendication 22, dans lequel le matériau composite comprend un mélange intime d'au moins un composé intermétallique de nickel-aluminium, d'au moins un composé intermétallique de nickel-aluminium-cuivre, d'oxyde de cuivre, et d'une solution solide d'au moins deux des métaux parmi le nickel, l'aluminium et le cuivre.

27. Le composant de cellule de la revendication 22, qui est une anode revêtue d'oxyfluorure de cérium.

28. Le composant de cellule de la revendication 22, qui est une cathode revêtue avec ou contenant au moins un borure de Métal réfractaire dur.

29. Le composant de cellule de la revendication 22, qui est imprégné d'oxyde de cérium, d'acétate de cérium, de silice, d'alumine, d'oxyde d'yttrium, d'oxyde de thorium, d'oxyde de zirconium, d'oxyde de magnésium ou d'oxyde de lithium colloïde.

30. Le composant de cellule de la revendication 22, dans lequel le cérium provenant du colloïde représente de 0,2 à 10 % en poids du matériau composite.

31. Précurseur d'un composant d'une cellule de production d'aluminium qui est allumable pour produire par réaction micropyrétique un composant de cellule réalisé avec un matériau composite comprenant au moins un composé d'aluminure ordonné d'au moins un parmi le nickel, le fer et le titane, dans lequel le précurseur est formé d'un mélange de réaction séché comprenant des réactifs particulaires compactés qui réagissent pour produire le matériau composite, les réactifs particulaires compactés étant mélangés avec et liés par le porteur colloïdal à base de cérium.

32. Le précurseur de la revendication 31, dans lequel le porteur colloïdal à base de cérium comprend au moins un parmi l'oxyde de cérium et l'acétate de cérium colloïdaux.

33. Le précurseur de la revendication 32, dans lequel le porteur colloïdal à base de cérium comprend au moins un parmi l'alumine, l'oxyde d'yttrium, la silice, l'oxyde de thorium, l'oxyde de zirconium, l'oxyde de magnésium, l'oxyde de lithium ou le monoaluminium phosphate colloïdaux.

34. Le précurseur de la revendication 31, obtenu par séchage d'un porteur colloïdal à base de cérium ayant un contenu de colloïde solide correspondant à jusqu'à 50 % en poids de porteur colloïdal, préférablement de 10 à 20 % en poids, ayant ainsi de 10 à 20 ml de porteur colloïdal par 100 grammes de mélange de réaction.

35. Le précurseur de la revendication 31, dans lequel le mélange de réaction comprend des métaux particulaires ou des composés de métaux sélectionnés du groupe consistant de l'aluminium, du nickel, du fer, du titane, du cuivre, du chrome, du manganèse, du vanadium, du molybdène, du zirconium, du niobium et du cérium, et leurs mélanges.

36. Le précurseur de la revendication 31, dans lequel le mélange de réaction comprend de 50 à 100 parts en poids d'au moins un parmi le nickel, le fer, et le titane particulaires, et de 2 à 50 parts en poids d'aluminium particulaire.

37. Le précurseur de la revendication 31, dans lequel le mélange de réaction comprend de 1 à 30 parts en poids d'additifs particulaires sélectionnés parmi le cuivre, le chrome, le manganèse, le vanadium, le molybdène, le zirconium, le niobium et le cérium et leurs composés ainsi que des composés d'aluminium, de nickel, de fer et de titane.

38. Le précurseur de la revendication 37, dans lequel le mélange de réaction comprend de 50 à 100 parts en poids de nickel particulaire, de 2 à 50 parts en poids d'aluminium particulaire et de 1 à 25 parts en poids de cuivre particulaire.

39. Le précurseur de la revendication 38, dans lequel le mélange de réaction comprend de 50 à 90 parts en poids de nickel particulaire, de 5 à 30 parts en poids d'aluminium particulaire, de 5 à 25 parts en poids de cuivre particulaire et de 0 à 15 parts en poids d'additifs sélectionnés parmi le chrome, le manganèse, le vanadium, le molybdène, le zirconium, le niobium et le cérium et leurs composés ainsi que les composés d'aluminium de nickel, de fer, de titane et de cuivre.

40. Le précurseur de la revendication 37, dans lequel le mélange de réaction comprend au moins un oxyde d'au moins un métal du groupe de l'aluminium, du titane, du cuivre, du chrome, du manganèse et du cérium.

41. Le précurseur de la revendication 37, dans lequel le mélange de réaction comprend au moins un métal du groupe du titane, du chrome, du vanadium, du zirconium, du niobium et du cérium, ou des précurseurs qui réagissent pour former lesdits borures.

42. Le précurseur de la revendication 31, dans lequel le matériau composite comprend au moins un composé intermétallique du groupe du AlNi, AlNi₃, Al₃Fe, AlFe₃, AlTi et AlTi₃ ainsi que leurs composés intermétalliques ternaires dérivés, et les solutions et mélanges solides d'au moins un desdits composés intermétalliques avec au moins un des métaux parmi l'aluminium, le nickel, le fer, le titane, le cuivre, le chrome, le manganèse, le vanadium, le molybdène, le zirconium, le niobium et le cérium et les oxydes desdits métaux.

43. Le précurseur de la revendication 31, dans lequel le cérium provenant du colloïde représente de 0,2 à 10 % en poids du matériau composite.

44. Mélange de réaction pour produire un composant d'une cellule de production d'aluminium, lequel composant est réalisé avec un matériau composite comprenant au moins un composé d'aluminure ordonné d'au moins un parmi le nickel, le fer et le titane, par réaction micropyrétique d'un mélange de réaction après séchage et compactage, le mélange de réaction comprenant des réactifs particulaires qui réagissent pour produire le matériau composite mélangé avec un porteur colloïdal à base de cérium dans une quantité d'au moins 5 ml de colloïde par 100 grammes du mélange de réaction.
